

June 5, 1928.

1,672,352

J. E. THORNTON

TWO-PLY CINEMATOGRAPH POSITIVE FILM

Filed May 4, 1926

2 Sheets-Sheet 1



Fig. 1.



Fig. 3.



Fig. 4.



Fig. 7.



Fig. 2.



Fig. 5.



Fig. 8.



Fig. 6.

Fig. 10.



Fig. 9.

INVENTOR.

J. E. Thornton  
J. O'Donnell  
attys.

June 5, 1928.

1,672,352

J. E. THORNTON

TWO-PLY CINEMATOGRAPH POSITIVE FILM

Filed May 4, 1926

2 Sheets-Sheet 2



Fig. 11.



INVENTOR.

J. E. Thornton  
by J. O'Conor O'Brien  
attn

## UNITED STATES PATENT OFFICE.

JOHN EDWARD THORNTON, OF WEST HAMPSTEAD, LONDON, ENGLAND.

## TWO-PLY CINEMATOGRAPH POSITIVE FILM.

Application filed May 4, 1926; Serial No. 106,731, and in Great Britain March 18, 1926.

This invention relates to an improved cinematograph two-color film of positive pictures, of the type built up from two thin films cemented together back-to-back, the 5 images upon one outer face of the completed film being of orange-red coloring and those upon the opposite outer face of blue-green coloring, one of the images being reversed in relation to the other; and to an 10 improved process of producing such film with silver sensitizing; without having to color or dye the two sets of images after printing; without having bare margins thinner than the rest of the film to prevent 15 creeping and mixing of the two dyes; without forming a softened weakened hinge longitudinally of the strip to enable it to be folded; without folding the strip; without the use of methyl-alcohol to soften the cel- 20 luloid backs; and without need for cementing the two thin films together before development; all of which features are used in the production of another two-color film of the two-ply type, but are not used in the 25 present invention.

The characteristic features of the present invention therefore comprises the following, used or operating in combination:-

- (1) Ready-colored film-material, of
- 30 (2) Double-width, with two parallel colored stripes,
- (3) Sensitized with silver for rapid printing;
- (4) Side-by-side development, without
- 35 folding or cementing the film;
- (5) Insoluble printed margins, retaining full strength and thickness of film-material;
- (6) Severing the strip after development and finishing and before cementing;
- 40 (7) True width without folding or trimming;
- (8) Joint formed by two layers of slow-drying cement;
- (9) Registration by special registration
- 45 perforations made before printing;
- (10) Traction by additional perforations made after printing, finishing and cementing;
- (11) Image-pair identification by numbers;
- 50 (12) Varnishing the finished print.

According to the invention the positives are printed upon a double-width strip of ready-colored film-material comprising two parallel stripes of orange-red and blue-green

colored colloid, carried upon and amalgamated by means of an adhesive substratum with a double-width support of transparent celluloid or like waterproof material, the thin film having a thickness approximately half the ultimate thickness of a completed film-positive, the colloid layer being sensitized with silver salts, preferably as a gelatino-silver emulsion. This film-material is printed by exposure from the back through the celluloid support and through a suitable printing-cliché of negative character, to produce a positive with relief images.

The colloid is gelatine, and the coloring matter may comprise pigments or dyes, but dyes are preferred and are suitably mordanted to prevent their washing out.

The film-material is printed, developed, and dried whilst in its double-width form, after which it is longitudinally severed to form two films that are subsequently cemented together back-to-back to form the completed single-width film-positive.

The accompanying drawings illustrate the invention in which drawings:-

Fig. 1 shows a strip of ready-colored double-width sensitized film of half standard thickness, orange-red on one half and blue-green on the other half.

Fig. 2 shows the same film perforated before printing with one hole for each picture component for registration purposes only while printing, assembling, and cementing.

Fig. 3 shows a double-width negative strip having the conventional design of a square, the image for one negative being reversed. The negative on the right represents orange-red and that on the left blue-green. Two single-width negatives may be used side by side instead of one double-width.

Fig. 4 shows the positive as it would appear after printing with the picture images alone, if developed without also printing the margin.

Fig. 5 shows the same positive after receiving a second exposure to print the margins so that the latter will be rendered insoluble and appear solid black after development.

Fig. 6 is a section through the developed positive, the images being represented by the colloid graduations and the margins by the solid black portions.

Fig. 7 represents the two pictures after the double-width film has been severed longitudinally and the two halves superimposed, registered by the two registration holes, and cemented.

Fig. 8 shows the finished film after perforation with the eight traction holes.

Fig. 9 is a perspective view of the two films being brought together for the cementing operation, the end of the figure showing the two celluloid centres, the two relief images in section, and the thick insoluble printed margins.

Fig. 10 shows an enlarged longitudinally section of a strip of sensitized film-material provided with a temporary paper backing which acts as a strengthening strip during the printing and developing operations.

Fig. 11 shows means for uniting the two films together.

The thickness of the various layers are approximately as follows:

The celluloid layer  $1, \frac{2}{1000}$  of an inch.

The substratum  $2, \frac{1}{10000}$  of an inch.

The colored sensitized colloid layer  $1, \frac{1}{1000}$  of an inch.

The temporary paper reinforcement  $2, \frac{1}{1000}$  of an inch, but in the various figures the printed colloid-relief-layer is shown enlarged out of proportion to the thickness of the other layers for the sake of clearness.

#### *Film-material and sensitizing process.*

The film-material may be of the type comprising a celluloid layer, a substratum layer, a colored colloid layer, and a temporary reinforcing strip of paper attached to its colored face for giving extra strength to the film during the printing and developing processes, as described in my specification Serial No. 35761, June 8th, 1925; or it may be of the non-reinforced ordinary type film-material comprising a celluloid layer, a substratum layer, and a colored colloid layer, as described in my specification Serial No. 35,760 June 8th, 1925. In both forms the film-material is provided with two parallel strips of colloid ready colored with the correct pair of colors, and with the correct quantity of color in each, that will produce a finished picture having properly balanced and proportioned colors without any need for the usual troublesome dyeing of the images or adjusting the colorings by the printer after the film has been exposed and developed, which are necessary with other processes. These two colors are orange-red and blue-green, but instead red and blue may be substituted upon condition

that after the film has been developed a yellow dye is applied all over the film in order to convert the red images into orange-red and the blue images into blue-green.

The film-material is sensitized with salts of silver by any of the known methods, but the method preferred is to use a gelatino-silver-bromide emulsion of the usual type, or a gelatino-silver-chloride emulsion, the emulsion being coated on to an adhesive substratum previously coated on to the cellulose support and dried this substratum effecting a perfect union or amalgamation of the support and emulsion, the colors being incorporated in the emulsion layer as aforesaid.

#### *Negatives, or printing clichés.*

The negatives used for printing may be either the original negatives or printing-clichés reproduced therefrom, and the two component negatives or clichés may be formed as two parallel rows upon a double-width strip, or two separate single-width negative-strips may be used side by side.

#### *Printing the positives.*

Printing of the double-width strip is effected in the same manner as in printing ordinary non-colored film, except that more exposure is necessary, which is preferably attained by using a more powerful lamp in the printing-machine. The printing-machine is also of standard type except that it is made to take a film of double-width.

Printing must be effected through the back of the film support, not from the face side, the negative also being reversed so that the images are right way about. That is to say, the celluloid sides of both films are towards each other during the operation of printing.

Printing can be effected either by contact or by the projection method, the latter being preferred. The negative film therefore passes through one machine in front of a lamp and the images are projected by means of either one lens (or a pair of lenses) on to the positive film, which passes through another machine placed opposite, the two machines being mounted upon a baseplate and geared to synchronize, the lens or lenses being mounted between. The light beams are made to take parallel form in order to ensure sharp images.

#### *Identifying components.*

To guard against any possibility of mistakes in correctly assembling the two component images of the same picture, identification numbers may be printed on both films.

#### *Margins of full strength and thickness.*

In other inventions where images are

formed in relief a characteristic feature has been that the margins of the film were bared and freed from gelatine after development and before coloring, which had the effect of 5 reducing the thickness of the finished cemented film at the perforated margins, thus considerably reducing the strength of the film at the very place where it most needed strengthening. These bare margins formed 10 dams, which prevented creeping and mixing if the two dyes during the process of dyeing the two sides of the printed and cemented film.

A feature of the present invention is that 15 this objection is removed by leaving the full thickness of gelatine covering both margins of both component strips, so that when the two films are cemented together the completed film-positive will have full thickness 20 and full strength at the two margins where most needed. This is rendered possible because it is not required to dye the two sides of the print after completion as they are already colored.

In the ordinary course of printing films 25 of the relief type the margins are covered by opaque parts of the printing-cliché, and receive no exposure and subsequent treatment to insolubilize them, and therefore dissolve away during the hot water development. But in the present invention these 30 margins are given a separate and very complete exposure and subsequent treatment, to render them completely insoluble, by exposing them to the printing lamps in such manner that the already exposed image parts are 35 protected by an opaque covering mask and the margins are left uncovered and exposed to the full light of the lamps thus producing 40 printed margins which on development remain solid, insoluble, and of full thickness.

A characteristic feature therefore of this 45 invention is that the margins of the printed films are always rendered insoluble and opaque or fully-colored, and are always left finished with the full thickness and strength of the original film-material.

#### 50 *Developing the positives.*

The positive images are developed in the ordinary way, preferably by machine; not only the developing but also the subsequent processes of treatment being carried out successively by means of different baths as the film progresses continuously through the machine.

Any suitable known developer may be used, such as metol-hydroquinone, pyrogallic acid, and others.

After development the film is treated in an oxydizing and bleaching bath of the usual type, by which the gelatine is hardened where in contact with the grains of metallic silver and in direct ratio to the amount of

such silver reduced by the developer. These portions of the gelatine where there is no metallic silver deposit remain soft and soluble.

The film is next fixed in a bath of sodium hyposulphite to which may be added a small proportion of an alkaline ferricyanide such as potassium-ferricyanide, and the whole of the silver (exposed and unexposed) is dissolved out of the film, leaving behind a transparent but colored gelatine body having images of hardened insoluble gelatine and other parts that remain soft and soluble.

The film is next dried to complete the hardening process, after which it is treated in a bath which is a solvent of soft gelatine. This may be hot water, or a cold strong solution of a bichromate salt, such as sodium bichromate, with or without the addition of a little acetic acid, or any other of the various solvents of gelatine. When all the soft gelatine has been dissolved and washed away a film is left with two parallel rows of images in relief, one of orange-red colored gelatine and the other of blue-green colored gelatine, and without silver or any other light-obstructing agent.

Development is now complete. No other operations are necessary. No subsequent dyeing of the images is required. The film is finally dried and is then ready for the cementing operations.

The entire operations of developing and drying may be effected by any suitable type of machine, one convenient form being that described in my Patent No. 1,173,895.

#### *Cementing after developing and finishing.*

In other inventions where images are formed in relief a characteristic feature has been that the two films were cemented together back-to-back (cellulose-to-cellulose) immediately after printing and before development, in order that the images upon opposite sides of the central support could be developed simultaneously in a hot water bath. They were not dyed until after development, and then each side was dyed separately.

But in the present invention the two films are printed, developed, washed, finished and dried whilst in their double-width form, and are not severed, superimposed and cemented until the whole of these several operations have been completed. This method presents many advantages in manufacture, one of which is that the wet prints are not injured upon their faces by contact with the numerous sprockets and other mechanism of the developing machine, but on the contrary are maintained face outwards with only the back of the celluloid support in contact with the machinery until the last printing and developing operation has been finished and the film-images dried.

*Producing without longitudinal weakening or folding.*

In another invention where two sets of images have been printed upon a double-width film, the film has been first longitudinally folded and doubled over upon a line midway between the two sections and then passed through a perforating machine which punched holes through the double thickness. The film was then unfolded and laid as flat as possible in order that it could be printed by contact with the printing cliché. Next it was again folded and cemented celluloid-to-celluloid prior to development, and finally the folded edge was cut away by a trimming machine. The objections to such a system are that the film-material needs to be wider to allow for trimming, and has to be reduced in thickness at the fold by the application of a partial solvent in order to make the film more pliable at the hinge, so that it can be folded more sharply, and also to enable it to be refolded or unfolded readily. This process has to be carried out whilst the film is sensitive, and before printing; and the treatment of sensitive film in this manner is objectionable in many ways as well as rendering the film liable to distortion owing to the solvent-produced hinge. In the present invention none of these objections apply, because the film is never folded but is perforated printed, developed, treated and dried and also longitudinally severed whilst in its original flat condition, and the two sections are always true to width, need no trimming, are without any liability to distortion, and the perforations are capable of accurately superimposing and registering.

*Separate registration and traction perforations.*

The perforations may comprise the usual four holes per margin per picture, which means sixteen holes for the pair. But I prefer to perforate the film before printing with only one hole per complete picture for registration purposes only. This means that two adjacent holes are formed in the central margin of the double-width film between the two rows of section pictures, one for each picture-component, and when the two severed single-width films are superimposed and cemented together these two holes coincide in accurate register and form only one hole in one margin of the completed picture. The united strip is next passed through a perforating machine which punches the set of eight holes per picture for traction purposes, four in each margin, using the hole already made as a pilot hole from which to work in positioning the remaining holes. This pilot hole may form one of the set of eight. Any other desired number of holes

or type of perforations may be used instead of the usual standard eight. This system is described in specification of my application Serial No. 66,605 filed November 5, 1925, and is particularly well suited for use in the 70 form of film comprising the present invention.

*Uniting by two slow-drying thin layers of cellulose.*

75

After printing and finishing the double-width film is slit into two strips as aforesaid and these are next united to form a single strip, with its two sets of images located upon its two opposite faces, by cementing the two thin strips back-to-back (cellulose-to-cellulose).

It is preferred not to slit the film until this last operation of cementing, and preferably by a rotary slitting knife which effects 85 the operation immediately before cementing, so that expansion and contraction will be uniform for both sections up to this last stage.

In other inventions it has been proposed 90 to unite two celluloid-films by softening their backs with methyl-alcohol, in order to effect a quick-union by employing a solvent that will speedily evaporate. It is well-known by those versed in the art of film manufacture 95 that the quicker a solvent evaporates the less secure will be the union of two cellulose faces joined by its aid.

In carrying out the jointing portion of this invention I therefore do not attempt 100 to make a quick joint by use of a quickly-evaporating solvent of the cellulose supports, but on the contrary I use a slow-drying cement of cellulose composition containing a heavy solvent that will not dry too rapidly. 105

The cement is preferably applied to the backs of the two films (whilst they are suitably supported and carried) by means of spreading knives, scrapers, or rollers that will apply an extremely thin measured layer 110 of definite thickness of the thick non-flowable paste-like cement-compound. Thus a separate layer of the cement is first laid upon the backs of the celluloid or other cellulosic supports. The cement very slowly partially penetrates the cellulose support, becomes amalgamated therewith as part of its body, and also forms a superimposed thin layer or film of cement which remains upon the surface as a layer of very great adhesiveness. 115 When therefore the two cement-coated backs of the two films are brought into contact and pressed together the two supports become amalgamated, as if only one strip, by means of the two extremely thin layers of cellulose paste, which eventually dry hard owing to gradual penetration of the solvent through the support and the assistance of heat during passing of the united films through a suitable drying chamber. 120 125 130

- This cellulose paste is of the kind often termed "dope" but is stiffer than the flowable variety used for casting film supports. The composition of the cement depends upon 5 the composition of the transparent support. If for example the support is of nitro-cellulose (commonly termed celluloid) the cement is made from dry cuttings of that material dissolved in amyl-acetate, which is a 10 comparatively heavy slow-drying solvent. If the support is one of the non-flam type, comprising one of the many varieties of cellulose acetate, the cement is made from dry cuttings of that material dissolved in the 15 heaviest solvent of that material. The particular solvent will vary according to the particular make of cellulose-acetate used; the variety of non-flam forms of cellulose are numerous, and a different slow-drying solvent is usually necessary with each variety. 20 It is usual in mixing cellulose cements to incorporate a large proportion of a quickly-evaporating solvent even where a slow-drying solvent is also used; but in the invention 25 I do not use or incorporate any of such highly-volatile solvents but instead rely entirely upon solvents that will slowly penetrate and amalgamate the films and will take considerable time to dry off.
- 30 During application of the thick paste-like cement to the backs of the two films they are suitably held and carried by a cementing registering and uniting machine, which draws the two films from two supply-spools, positions them with fair accuracy by 35 means of sprocket wheels the teeth of which engage with the perforations of the films; the cement is applied in a thin layer or film by scrapers or rollers as the films travel through this machine; and finally the two 40 films are brought into near juxtaposition, and are then engaged by pins which accurately register the two component images, the pins, exactly filling the perforations of 45 the films, and then the two films are clamped between reciprocating clamping blocks by which they are squeezed together and completely united. Owing to the slow-drying and very adhesive cement used a comparatively 50 light pressure only is needed for this part of the operation.
- The mechanical methods of carrying out this part of the process, and machines therefor, are described in my Patent No. 1,169,- 55 098 and of application Serial No. 756,168, filed December 15, 1924.
- One such machine is illustrated in Fig. 11. The stiff cellulose paste or dope is contained in the hoppers A from which it falls 60 through a slit B, the thickness of the layer of paste applied to each film being exactly determined by a scraper knife C controlled by a screw c. Each film is drawn over a spreading table D and the slits B are arranged sufficiently far back from the point 65 where the two films come together to give the paste time to partially amalgamate with the film-supports before they are registered and squeezed together by the blocks E. The films pass from the tables D over the 70 sprocket wheels D<sup>1</sup> to the first pair of movable cementing blocks E which are provided with registration teeth and thence to the final movable blocks D<sup>1</sup>.
- The method of uniting the two films previously described has the advantage that the films to be united remain comparatively dry and stout whereas if a fluid solvent such as methyl-alcohol alone is employed the 75 films become soft and liable to distortion. 80
- The two-color positive film is now complete and ready for exhibiting.
- If it is desired to vary the physical condition of the colloid images the film may be passed through a bath containing a very 85 small proportion of glycerine to keep the body of the colored colloid more supple and less hard. Or the bath may contain a very small proportion of chrome alum to harden the surface. I prefer, however, to apply to 90 the two surfaces of the completed film an extremely thin layer of a colloid varnish in which the glycerine and/or chrome alum are incorporated. This is effected by passing the finished film through a bath of these 95 combined ingredients, then past air jets which blow through the perforations to keep them clear of varnish, and finally drying the finished film.
- 100
- Summary.*
- The methods herein described for manufacturing a two-color cinematograph series of film-positives from ready-colored film-material, as a single film built-up from two 105 films that are cemented back-to-back (cellulose-to-cellulose) with the two component images located upon the two outer faces of the central support and in accurate register, produce a film with strong solid margins of full thickness, without any troublesome weakened fold, with less labour and fewer operations, without waste due to trimming, with a much better joint, and without the troublesome operations involved in 110 dyeing the two sides with two different colors after making the two prints, and represent considerable improvement upon the methods hitherto known and used.
- 115 What I claim as my invention and desire 120 to protect by Letters Patent is:—
1. A two-colour positive cinematograph film comprising in its construction two transparent supports of the exact width of the film, a layer of slow drying stiff cellulose 125 cement paste by which the supports are joined together, a layer of coloured colloid with images printed in relief in silver salts on each support, and insoluble solid margins at each edge formed of the printed col- 130

loid to the full thickness of the film material.

2. The method of producing a two-colour positive cinematograph film which consists in utilizing a transparent support coated with two stripes of differently coloured colloid one coloured orange-red and the other blue-green sensitized with silver salts printing thereon images in relief and printing the margins adjacent to the images to render them insoluble and solid of the full thickness of the film, developing and finishing the images, severing the support into two longitudinally the exact width of the film and cementing the supports together with a layer 15 of cellulose paste.

3. The method of producing a two colour positive cinematograph film as in claim 1 by printing the margins of sensitized colloid to produce solid insoluble margins of 20 full thickness equal to the original film.

4. The method of producing a two colour positive cinematograph film which consists in printing and producing images in relief upon a double width transparent support in

two parallel stripes of different coloured colloid sensitized with silver salts, submitting the margins at each side of the images to light to render them insoluble, severing the support longitudinally into two strips of exact width for the film and superimposing them upon two layers of cellulose paste by 25 which they are united back to back.

5. In the production of a two colour positive cinematograph film as in claim 1 subjecting the non-picture margins to a further exposure to light to render them insoluble and at the same time projecting the previously exposed picture portions of the film during the subsequent exposure by a covering mask which does not cover the margins. 30

6. A two colour positive cinematograph film as in claim 1 perforated along the solid insoluble margins substantially as described.

In testimony whereof I have hereunto set 45 my hand.

JOHN EDWARD THORNTON